

1

2,833,706

ELECTROLYTIC METHOD OF PRODUCING  
TITANIUM

Eugene Wainer, Cleveland Heights, Ohio, assignor, by  
mesne assignments, to Horizons Titanium Corporation,  
Princeton, N. J., a corporation of New Jersey

No Drawing. Application May 16, 1956  
Serial No. 585,172

7 Claims. (Cl. 204—64)

This invention relates to the production of lower valent halides of certain polyvalent transition metals from which the metals themselves may be obtained either by subsequent disproportionation of the lower valent metal halide or by electrolytic decomposition of the lower valent metal halide while dissolved in or assimilated by a fused salt bath.

Because of the possibilities inherent in the production of various transition metals either by electrolytic decomposition or by disproportionation of their lower valent halides, considerable attention has been devoted heretofore to the production of these lower valent halides. For this purpose, numerous reducing agents such as hydrogen and various metals have been proposed and used, but it has been characteristic of such procedures that a significant portion of the halogen component of the initial transition metal halide has been lost by its combination with the reducing agent. Consequently, the amount of lower valent transition metal halide thus produced has always been less than the starting amount of the higher valent transition metal halide. The use of the transition metal itself as a reducing agent has been proposed and explored, but the inherent disadvantage in this procedure is that it is predicated upon the previous production of the transition metal itself.

I have now discovered that the lower valent halides of the multivalent transition metals: titanium, zirconium, hafnium, vanadium, niobium and tantalum may be obtained by reaction between the higher valent simple halides of the metals and the lower valent sulfides of these metals. The method of my invention for producing the lower valent halides of these metals comprises bringing the higher valent simple halide of the metal in the vapor state into contact with a mass of the lower valent sulfide of one of these metals in the form of particles at least as fine as about 200 mesh, and effecting reaction between the higher valent metal halide and the lower valent sulfide by maintaining the reactants at a temperature at least as high as the volatilization temperature of the higher valent metal halide but below that at which the resulting lower valent metal halide disproportionates to the metal itself. I have further discovered that if the resulting lower valent transition metal halide is supplied to a suitable fused salt bath and is subjected to an electrolysis therein, the combination of these steps results in a process wherein the transition metal sulfide is converted to the transition metal itself without consumption of the transition metal higher valent halide.

The higher valent halides of the aforementioned transition metals useful in practicing the invention comprise the simple chlorides, bromides, iodides or fluorides provided that they are sufficiently volatile to permit their reaction with the lower valent sulfide in the substantially dry state, i. e., in the substantial absence of a molten phase, at temperatures below those at which the corresponding lower valent halide disproportionates. In general, these higher valent halides which are readily volatile are the tetra-

2

valent halides, although in the case of vanadium, higher valent halides such as the pentavalent halides are available. All of these metal halides are available in a state of purity adequate for the practice of my invention, but if desired, these halides may be further purified by distilling or subliming them into the reaction zone, or by any other appropriate purification procedure.

The transition metal sulfide used in the practice of my invention should be of high purity; that is, it should be free of contaminants which would otherwise be carried over into the lower valent halide product. High purity transition metal sulfides can be produced either by reacting the transition metal halides with hydrogen sulfide at appropriate elevated temperatures or by heating the impure transition metal with elemental sulfur under a controlled atmosphere. In the event that the metal is one which combines to form more than one sulfide, the transition metal sulfide selected should be one in which the transition metal exhibits a lower valence than the maximum valence of the transition metal. For example, in the case of titanium, three sulfides are known, namely, titanium disulfide, titanium sesquisulfide, and titanium monosulfide. In the practice of my invention only the latter two sulfides may be used, and where a divalent titanium halide is to be obtained, only the divalent sulfide, titanium monosulfide can be used.

In general, whatever the transition metal sulfide employed, it should be chosen from sulfides in which the valence of the transition metal is no higher than the valence of the transition metal in the lower valent transition metal halide to be produced.

The transition metal sulfide should be in a finely divided form in order to promote reaction between the sulfide and the transition metal higher valent halide. In general, I have found it advisable to use a sulfide particle size at least as fine as about 200 mesh (Tyler Standard). The reaction between the higher valent transition metal halide and the transition metal sulfide takes place readily at elevated temperatures when the vapors of the halide are passed over or through a mass of the finely divided sulfide. The reaction vessel, such as a quartz-lined furnace, should be gas-tight so that its atmosphere may be evacuated, then flushed with an inert gas such as argon and finally re-evacuated prior to the introduction of the transition metal higher valent halide. The reaction vessel is also advantageously provided with an outlet communicating with a closed condensing system in which the lower valent transition metal halide product may be liquified or solidified if the reaction temperature is above the normally liquid or solid state of the lower valent halide product.

The reaction temperatures at which the lower valent halides of the aforementioned polyvalent transition metals may be produced by the practice of my invention range between 300° and 1100° C., although the optimum temperature range for the production of the lower valent halides of the individual transition metals generally encompasses a narrower temperature range within this overall temperature range. In each instance, the reaction temperature should be at least as high as the volatilization temperature of the higher valent metal halide but below that at which the resulting lower valent halide disproportionates to the metal itself. Thus, effective reaction temperature ranges are as follows:

|           | ° C.           |
|-----------|----------------|
| Niobium   | About 400-900  |
| Tantalum  | About 400-900  |
| Titanium  | About 300-800  |
| Vanadium  | About 300-800  |
| Zirconium | About 600-1100 |
| Hafnium   | About 600-1100 |

Within each of these ranges, higher temperatures promote

more rapid reaction rates for each specific halide-sulfide reaction. In reactions wherein the lower valent halide product is not normally solid or liquid, increased pressure in the reaction zone will permit the use of a higher operating temperature while maintaining the same equilibrium as that prevailing at lower temperature and normal pressure. Accordingly, superatmospheric pressures may be used advantageously in the reaction zone in order to promote more rapid rate of the conversion of the higher valent transition metal halide to the lower valent halide.

The lower valent transition metal halide produced by the practice of my invention is generally the trivalent halide, although this halide is frequently accompanied by other lower valent halides. Within the effective operating temperature range for each transition metal halide, lower temperatures tend to promote the formation of halides having a lower valence than the halides produced at the higher operating temperatures. For example, in producing the lower halides of titanium from the tetrahalides of titanium, titanium trihalide formation is favored by reaction temperatures of about 400°-600° C.; but by lowering the temperature below this normal operating range for these metal halides, that is, by using a temperature of about 200°-350° C. at subatmospheric pressure, the dihalide predominates in the reaction product. Thus, by using a temperature range near or even below the optimum temperature ranges set forth hereinbefore, and by further using subatmospheric pressures, the reaction may be made to proceed effectively with the production of the lowest valent halides of each polyvalent transition metal, although generally, this result is achieved at the expense of lower reaction efficiency.

The following examples are illustrative of the practice of my invention for the production of lower valent halides of the aforementioned transition metals.

#### Example I

A silica tube furnace, equipped with a vacuum-tight water cooled head was used as the reaction vessel. A boat containing 200 gms. of 200 mesh high purity titanium monosulfide was inserted in the furnace and the unit was sealed and evacuated. The furnace was heated to a temperature of about 550° C. and titanium tetrachloride was then distilled into the reactor at a rate sufficient to maintain a reaction zone pressure of about one atmosphere. After four hours at 750° C., the furnace was cooled while maintaining a titanium tetrachloride pressure of one atmosphere until the furnace temperature was below the normal boiling point of titanium tetrachloride. The furnace was then opened, and the reacted mass was removed and leached with aqueous 1 N hydrochloric acid. After filtration, an aqueous solution of pure titanium trichloride was obtained.

#### Example II

The reaction was conducted as in Example I until the cooling stage was reached. At this time the flow of tetrachloride was stopped, argon was introduced into the furnace to flush out any gases present, and the furnace was evacuated to a pressure of  $10^{-2}$  atmosphere and cooled. The reaction mass contained titanium dichloride and titanium trichloride together with sulfur and unreacted titanium sulfide. The titanium chloride product was recovered in a form suitable for the electrolytic production of titanium by leaching the reaction product mass with a molten mixture of sodium chloride and potassium fluoride.

#### Example III

The reaction described in Example I was conducted in a quartz lined bomb. Liquid titanium tetrabromide and titanium monosulfide were sealed in the bomb, which was then heated to 450° C. A mixture of titanium dibromide and tribromide was obtained.

#### Example IV

200 grams zirconium sulfide and zirconium tetrachloride were reacted as described in Example I. The reaction temperature was held at about 800° C. Substantially a 100% yield of zirconium trichloride was obtained (1950 grams).

The lower valent transition metal halides produced by the practice of my invention may be used as a source of the transition metal supply for fused salt bath electrolytic production of the transition metal itself which results in a process wherein the transition metal sulfide is converted to the metallic state. The production of the lower valent halides can be visualized by the following representative equations in which M represents the transition metal, X represents a halogen and S is sulfur:



Regardless of which reaction course is actually representative of the combination of steps by which I produce the transition metal halide, it will be seen that the reactions involve the conversion of the higher valent transition metal halide to a lower valent halide which may be recovered in any suitable manner and then decomposed by a fused salt electrolysis.

The following examples are illustrative of the over-all process for converting one of the aforementioned transition metal sulfides to the form of the metal itself.

#### Example V

A boat containing 200 grams of minus 200 mesh (Tyler Standard) high purity titanium monosulfide was inserted in a silica tube furnace equipped with a vacuum tight, water cooled head. The furnace was sealed and evacuated. After the furnace was brought up to a temperature of about 550° C. titanium tetrachloride was admitted to the furnace reaction zone at a rate sufficient to maintain the pressure in the reaction zone at about one atmosphere, and the temperature of the furnace was raised to about 750° C. After four hours at 750° C., the furnace was cooled to about 100° C. while maintaining an atmosphere of titanium tetrachloride therein. The solid reacted mass was removed and leached with molten sodium chloride. Sufficient sodium chloride was employed to dissolve substantially all of the titanium di- and trichloride which formed and a melt containing upwards of about 93% by weight of sodium chloride was thereby produced.

The molten halide mixture was charged into an electrolytic cell provided with the usual means known in the art for maintaining the desired temperature, pressure, and atmosphere in the cell. The electrolysis of the molten chloride bath was carried out employing a graphite anode and a nickel cathode at a cell voltage of 1.6 volts and a cathode current density of 100 amperes per square decimeter. A finely crystalline deposit of metallic titanium was obtained on the cathode weighing 470 grams. Analysis of the residue obtained by leaching of the reaction mass with NaCl indicated a metal recovery of 93% based on the initial TiS and that the product was  $\frac{2}{3}$   $TiCl_3$  and  $\frac{1}{3}$   $TiCl_2$ .

#### Example VI

The molten mixture obtained by leaching the reaction product of Example II in the manner described, was charged into an electrolytic cell and electrolyzed therein at a cell voltage of 3.0 volts and a cathode current density of 100 amperes per square decimeter for a period of 100 minutes. The titanium chlorides therein contained were electrolytically decomposed and a deposit of 470 grams of titanium was obtained on a molybdenum cathode, representing a metal recovery of about 93%.

#### Example VII

Example V was repeated except that the electrolysis bath was prepared by leaching the reaction mass of Ex-

ample IV with molten sodium chloride. In the ensuing electrolysis, 850 grams of the zirconium were recovered as a cathode deposit. The electrolysis was carried out at 875° C., at 1.9 volts and 100 amperes per square decimeter of cathode area. The metal yield was 94.5%.

Although the practice of the invention has been described and illustrated hereinbefore for the production of the lower valent halides of a single polyvalent transition metal, as well as for the production of the individual metal itself, the process of the invention is equally applicable to the production of lower valent halides of a mixture of transition metals and, hence, to the production of mixtures or alloys of these transition metals. This result can be achieved either by using a higher halide of one transition metal and the sulfide of another transition metal, or by the use of either a mixture of the higher valent halides of two or more transition metals or of the sulfides of two or more transition metals, or by a combination of these procedures. The final metallic product can therefore be either the substantially pure transition metal itself or a mixture of two or more of these metals.

Furthermore although the foregoing specification has exemplified the preparation of lower valent halides of the several polyvalent transition metals by reaction between their simple higher valent halides (e. g.  $TiCl_4$ ,  $ZrCl_4$ ,  $VCl_4$ ,  $VF_5$ ) and their simple sulfides, it is to be noted that similar reactions may be effected between the simple sulfides and the complex higher valent halides of these metals, such as the double halides of the transition metal and an alkali metal, in which the transition metal exhibits one of its higher valent states. Thus  $K_2TiCl_6$ ,  $Na_2TiCl_6$ ,  $K_2TiF_6$  or  $Na_2TiF_6$  or other suitable complex tetrahalides of titanium may be substituted for the  $TiCl_4$  of Examples I or II, with similar results. Or complex titanium-alkali metal-bromides and complex zirconium halides in which the zirconium is tetravalent may be substituted in Examples III and IV without materially changing the processes disclosed.

It is also possible to carry out the same reactions (with little or no change in the reaction conditions) between complex halides of the polyvalent transition metals and complex sulfides of the transition metals to produce lower valent simple or complex halides of the metals from which the metals themselves may be recovered by a fused salt electrolysis in the manner of Examples V, VI and VII, above.

Accordingly, in the following claims the terms "halide" and "sulfide" are intended to include both the simple and complex transition metal halides or sulfides as the case may be, unless designated as one or the other, specifically.

Having now described my invention in accordance with the patent statutes, what I desire to claim is:

1. The method of producing a metal of the group consisting of vanadium, niobium, tantalum, titanium, zirconium and hafnium by electrolyzing a fused salt melt containing a lower valent halide of said metal which comprises: bringing a halide vapor of said metal in which the valence of the metal is higher than the valence of the metal in the lower valent halide to be electrolyzed into contact with a sulfide of one of said metals in the form of particles at least as fine as about 200 mesh the valence of the metal in the sulfide being no higher than the valence of the metal in the resulting lower valent product, effecting reaction between said halide vapor and said solid sulfide by maintaining the reactants at a temperature at least as high as the volatilization temperature of said higher valent metal halide but below that at which the resulting lower valent metal halide disproportionate to the metal itself, recovering the lower valent transition metal halide from the reaction mass by extracting same with at least one molten alkali metal halide, and electrolyzing the molten product containing the recovered lower valent transition metal halide whereby the transition metal is obtained as a cathode deposit.

2. The method of producing a metal of the group consisting of vanadium, niobium, tantalum, titanium, zirconium and hafnium by electrolyzing a fused salt melt containing a lower valent halide of said metal which comprises: bringing a higher valent halide of said metal in the vapor state into contact with a sulfide of one of said metals in the form of particles at least as fine as about 200 mesh, the valence of the metal in said halide being higher than the valence of the metal in the lower valent halide to be electrolyzed and the valence of the metal in the sulfide being no higher than the valence of the metal in the resulting lower valent halide product, effecting reaction between said halide and said sulfide at subatmospheric pressure by maintaining the reactants at a temperature at least as high as the volatilization temperature of said higher valent metal halide but below that at which the resulting lower valent metal halide disproportionate to the metal itself at said subatmospheric pressure, recovering the lower valent transition metal halide from the reaction mass by extracting same with at least one molten alkali metal halide, and electrolyzing the molten product containing the recovered lower valent transition metal halide whereby the transition metal is obtained as a cathode deposit.
3. The method of producing a metal of the group consisting of vanadium, niobium, tantalum, titanium, zirconium and hafnium by electrolyzing a fused salt melt containing a lower valent chloride of said metal which comprises: bringing a higher valent chloride of said metal in the vapor state into contact with a sulfide of one of said metals in the form of particles at least as fine as about 200 mesh, the valence of the metal in said chloride being higher than the valence of the metal in said lower valent chloride to be electrolyzed and the valence of the metal in the sulfide being no higher than the valence of the metal in the resulting lower valent chloride product, effecting reaction between said halide and said sulfide by maintaining the reactants at a temperature at least as high as the volatilization temperature of said higher valent metal halide but below that at which the resulting lower valent metal halide disproportionate to the metal itself, recovering the lower valent transition metal halide from the reaction mass by extracting same with at least one molten alkali metal halide, and electrolyzing the molten product containing the recovered lower valent transition metal halide whereby the transition metal is obtained as a cathode deposit.
4. The method of producing titanium which comprises: bringing titanium tetrachloride in the vapor state into contact with a sulfide of titanium in the form of particles at least as fine as about 200 mesh, effecting reaction between said tetrachloride and said sulfide by maintaining the reactants at a temperature at least as high as the volatilization temperature of said tetrachloride but below that at which the resulting di- and tri-chlorides disproportionate to the metal itself, recovering the di- and tri-chlorides from the reaction mass by extracting same with at least one molten alkali metal halide, and electrolyzing the molten product containing the recovered titanium chloride whereby the transition metal is obtained as a cathode deposit.
5. The method of producing titanium which comprises: bringing titanium tetrachloride vapor into contact with a sulfide of titanium in the form of particles at least as fine as about 200 mesh, effecting reaction between said vapor and said sulfide at subatmospheric pressure by maintaining the reactants at a temperature at least as high as the volatilization temperature of said tetrachloride but below that at which the resulting di- and tri-chlorides disproportionate to the metal itself at said subatmospheric pressure, recovering the di- and tri-chlorides from the reaction mass by extracting same with at least one molten alkali metal halide, and electrolyzing the molten product containing the recovered titanium chloride whereby the transition metal is obtained as a cathode deposit,

6. The method of producing titanium which comprises: bringing a tetrahalide of titanium in the vapor state into contact with a titanium sulfide of the group consisting of titanium monosulfide and titanium esquisulfide in the form of particles at least as fine as about 200 mesh, effecting reaction between said vapor and said sulfide by maintaining the reactants at a temperature at least as high as the volatilization temperature of said tetrahalide but below that at which the resulting di- and tri-halides disproportionate to the metal itself, recovering the di- and tri-halides from the reaction mass by extracting same with at least one molten alkali metal halide, and electrolyzing the molten product containing the recovered di- and tri-halides whereby the transition metal is obtained as a cathode deposit.

7. The method of producing titanium which comprises: bringing titanium tetrachloride vapor into contact with

a titanium of the group consisting of titanium monosulfide and titanium sesquisulfide in the form of particles at least as fine as about 200 mesh, effecting reaction between said tetrachloride and said sulfide at subatmospheric pressure by maintaining the reactants at a temperature at least as high as the volatilization temperature of said tetrachloride but below that at which the resulting di- and tri-halides disproportionate to the metal itself at said subatmospheric pressure, recovering the di- and tri-halides from the reaction mass by extracting same with molten sodium chloride, and electrolyzing the molten product containing the recovered lower valent titanium halide whereby the transition metal is obtained as a cathode deposit.

No references cited.